

April 6, 1965

W. C. SIEVERT

3,177,088

GALVANIZED STEEL MATERIAL AND PROCESS FOR PRODUCING SAME

Filed April 28, 1961

2 Sheets-Sheet 1



Inventor:  
William C. Sievert,  
By Norman, Smith, & Marshall,  
Atty's.

April 6, 1965

W. C. SIEVERT

3,177,088

GALVANIZED STEEL MATERIAL AND PROCESS FOR PRODUCING SAME

Filed April 28, 1961

2 Sheets-Sheet 2

Fig. 4.



Inventor:  
William C. Sievert,  
By Merriam, Smith & Marshall,  
Attn: J. S.

1

3,177,088

GALVANIZED STEEL MATERIAL AND PROCESS  
FOR PRODUCING SAMEWilliam C. Sievert, Chesterton, Ind., assignor to Inland  
Steel Company, Chicago, Ill., a corporation of Delaware

Filed Apr. 28, 1961, Ser. No. 106,324

19 Claims. (Cl. 117—66)

The present invention relates generally to galvanized steel material and more particularly to galvanized steel material having a smooth dark gray coating which is readily paintable, which is highly adherent to the steel base, and which has excellent corrosion-resistant properties; and to a process for producing this material.

Essentially, the subject material is produced by heating galvanized steel material to a temperature at which Fe from the steel base alloys with the Zn in the coating and until the iron content at the outer surface of the coating is at least about 7%. This alloying step may be carried out immediately after the zinc coating has been applied and while the zinc coating is still molten; or it may be carried out at any time after the galvanized material has cooled following coating.

The coating on the subject material has a smooth, dark gray, spangle-free appearance. The iron content of the coating varies from the outer surface of the coating to the interface between the coating and the steel base and is characterized by a concave curve in the plot of iron content versus distance from the outer surface of the coating. The varying iron content and the shape of the iron gradient curve can be determined by X-ray spectroscopic analysis or other methods well known to those skilled in the art.

It is essential that the coating have an iron gradient characterized by the concave curve described above. If the curve departs from a concave line the adherence properties of the coating become poorer, eventually resulting in a relatively brittle dark gray coating as the curve approaches a convex line. It has been discovered that a brittle dark gray coating is an indication that sufficient alloying has not taken place. Accordingly, the brittleness can be eliminated and the material salvaged by subjecting the material to an additional alloying treatment, said salvaging constituting a feature of the present invention.

The smooth, spangle-free, adherent, relatively ductile dark gray coating on the subject galvanized material renders this material ideal for painting purposes. No preliminary processing is required to condition this material to receive a coating of paint. It is possible that the dark gray color of the coating might be considered objectionable if the galvanized material were to be used in an unpainted condition. However, since the material is intended for painting purposes, the color of the coating is of no particular concern.

The dark gray coating of the subject material also possesses superior corrosion-resistance properties, as exemplified by an inability to readily strip this coating with a 50%, by weight, HCl stripping solution. The corrosion-resistance properties of this coating are better than those of the light gray coating described in U.S. Letters Patent No. 3,056,694.

Other features and advantages of the subject invention will become apparent to those skilled in the art from the following detailed description in conjunction with the accompanying drawings wherein:

FIGURE 1 is a diagrammatic view of one embodiment of a process for producing the subject material;

FIGURE 2 is a fragmentary diagrammatic view illustrating another embodiment of a process for producing the subject material;

2

FIGURE 3 is a diagrammatic view of a third embodiment of a process for producing the subject material; and

FIGURE 4 is a graph showing the iron content curves for coatings on various galvanized steel materials.

With reference to the process illustrated diagrammatically in FIGURE 1, a strip of steel material 10 from a coil 11 is initially passed through an oxidizing furnace 12 to produce a thin film of oxide coating on the surface of the steel strip. Strip 10 is then passed through a reducing furnace 13 which causes a reduction of the oxide coating on the surface of the steel and the formation of a tightly adherent impurity-free surface layer of metal on the steel strip. The strip 10 is then passed over an idler roller 14 and through a hood 15 into a zinc bath 17 contained in a dip pot 16 wherein a coating of zinc is applied to the surface of the steel strip. The steel strip is moved around an idler roller 18 in dip pot 16 and then upwardly through a pair of thickness-regulating rollers 19 which control the thickness of the coating on the strip. Up to and including the thickness-regulating step the process is conventional and is described in greater detail in U.S. Patent No. 2,110,898, issued March 15, 1938.

In accordance with the present invention, the steel strip coated with a layer of zinc is then subjected to an alloying treatment by moving the strip through a furnace 20. Performing the alloying step immediately after the coating step capitalizes on the zinc coating still being in a substantially molten state, thereby facilitating alloying between the iron and the zinc, and accordingly cutting down the length of furnace needed to produce the desired amount of alloying.

Following the alloying step, the galvanized strip is cooled by artificial cooling means 21 such as a water spray chamber, or allowed to cool in air, and then moved over a roller 22 and wound into a coil 23.

The temperature in the alloying furnace 20 and the length of time for which the galvanized strip must be exposed to the alloying temperature vary in accordance with the thickness of the strip and the thickness of the zinc coating thereon. For purposes of illustration, it is assumed that the strip has a thickness of 14 to 24 gauge with a zinc coating of 0.5—1.5 ounces (preferably 0.7 to 0.9 ounce) of zinc per square foot. The desired coating can then be obtained if furnace 20 is maintained at a temperature of about 1800° F. to 1900° F. and if the strip is moved through the furnace at a speed which subjects the strip to these temperatures for a period of about 60 seconds. The resulting material has an Fe content at the outer surface of the zinc coating in excess of 7% by weight, and an Fe gradient curve characterized by the concave shaped curve C in the graph of FIGURE 4 which plots Fe content against distance from the outer surface of the coating.

Furnace 20 may be a conventionally constructed continuous heat treatment furnace of a type well known to those skilled in the art, and may include conventional damper means or the like for admitting controlled amounts of air into the furnace to avoid non-oxidizing conditions therein, said non-oxidizing conditions tending to retard the alloying between the iron and the zinc.

The subject material may also be produced by the process illustrated diagrammatically in FIGURE 2. In this embodiment the galvanized strip is wound into a coil 23 following the coating step. A plurality of these coils 23 are then placed inside a conventionally constructed box-type annealing furnace 24 and heated until the desired amount of alloying has taken place. Assuming the galvanized material has a base material gauge and coating thickness similar to those described above with reference to the process illustrated in FIGURE 1, the desired coating can be provided by holding the coils at

a temperature of 1200° F. for about 2 to 5 minutes, followed by cooling in air; or by heating to about between 1000° F. and 1100° F. and holding for a period of about 5 minutes, followed by cooling in air. Lower alloying temperatures require longer periods of time at the alloying temperature. For example, if the alloying temperature is below the melting point of zinc (e.g., 750° F.) the time required to insure the necessary alloying may be several hours.

It should be noted that there is no harm in exposing the galvanized material to alloying temperatures for periods beyond the minimum period necessary to produce the desired amount of alloying. In other words, if the minimum time for producing the desired amount of alloying at a low temperature such as 750° F. is 48 hours, no harm can be done by subjecting the material to this alloying temperature for periods exceeding 48 hours. This is perhaps best illustrated by referring to curves A and B in the graph of FIGURE 4. Curve A illustrates the iron gradient curve for material subjected to an alloying temperature of 750° F. for a period of 48 hours, whereas curve B is the iron gradient curve for material subjected to this same temperature for 72 hours. Both curves have the characteristic concave shape indicating that their respective coatings are endowed with the desired properties. The only difference is that the coating characterized by curve B has a higher iron content throughout its thickness. More specifically, the coating of curve A has an Fe content varying from about 8% at the coating outer surface to 50% at the interface, whereas the Fe content in the coating of curve B varies from 20% at the outer surface to 50% at the interface.

FIGURE 3 illustrates a third embodiment of a process which may be utilized to produce the subject material. In this embodiment the galvanized strip is initially heated in a continuous type annealing furnace, then wound into a coil 23, following which the coils 23 are subjected to further alloying in a batch type box furnace 24. A process utilizing two alloying steps eliminates the construction of expensive extensively lengthy continuous type annealing furnaces 20. This type of process can also be used to salvage galvanized material having dark gray coatings which are brittle. Brittle dark gray coatings may be the result of under-alloying during a process intended to produce the subject material; or of over-alloying during a process intended to produce the light gray-coated material described in U.S. Letters Patent No. 3,056,694, referred to above.

Curve D in FIGURE 4 illustrates the iron content curve for a galvanized material having a brittle dark gray coating. By subjecting this material to a salvaging treatment constituting additional alloying, the configuration of the curve can be changed from the convex type illustrated by curve D to the concave type illustrated by curves A and B. The coating on the salvaged galvanized material has the same desirable characteristics as the coating on material not requiring the salvaging treatment.

When coils of galvanized material undergo alloying treatment by heating in box-type furnaces, the coils may be tightly wound or they may be of the "open coil" type with each of the turns of the coil spaced from the others by thin separators. Open coil heating is disadvantageous in that it takes less time and in that the alloying is more uniform. Tightly wound coils experience more alloying in the outer turns than in the inner turns of the coil, but this need not be deleterious if alloying is continued until the inner turns have an iron gradient curve such as that of curve A in FIGURE 4. Under these circumstances the outer turns of the coil would have a curve somewhat similar to curve B in FIGURE 4. Both inner and outer turns would have adherent, corrosion-resistant, dark gray coatings, because every turn of the coil would have a coating with an iron gradient characterized by a concave

curve, and because every turn of the coil would have an iron content at the outer surface of the coating greater than 7%.

There have thus been described typical processes for producing galvanized steel material having a smooth, spangle-free, tightly adherent dark gray coating ideally suited for painting. It should be understood that the subject invention is not limited to material produced by continuous-type galvanizing processes. Batch-type processes or other processes well known to those skilled in the art would be equally applicable, the important thing being that the galvanized material is subjected to an alloying step following the galvanizing step, which alloying step produces a coating having an iron content at the outer surface of the coating in excess of 7% and having an iron gradient characterized by a concave type curve as illustrated in FIGURE 4. The subject invention also enables the salvaging of galvanized steel material having a brittle dark gray coating.

The foregoing detailed description has been given for clearness of understanding only, and no unnecessary limitations should be understood therefrom, as modifications will be obvious to those skilled in the art.

I claim:

1. A process for producing an adherent, corrosion-resistant, dark gray galvanized coating on flat steel material, said process comprising the steps of:

coating flat steel material having a thickness of about 14-24 gauge with about 0.5-1.5 ounces of zinc per square foot; and then alloying said zinc in said coating with iron from said steel material by heating said zinc-coated steel material at an iron-zinc alloying temperature between 750° F. and 1900° F. for a time between 60 seconds and 72 hours.

2. A process as recited in claim 1 wherein said zinc-coated steel material is heated at an alloying temperature of about between 1800° F. and 1900° F., while said coating is still in a substantially molten condition, for around 60 seconds.

3. A process as recited in claim 1 wherein said zinc-coated steel material is heated at a temperature between 1000° F. and 1900° F. for a time between 60 seconds and 5 minutes.

4. A process as recited in claim 1 wherein said zinc-coated steel material is heated at a temperature between 1000° F. and 1200° F. for a time between 2 minutes and 5 minutes.

5. A process as recited in claim 1 wherein said zinc-coated steel material is heated at a temperature between 750° F. and 1000° F. for a time between 5 minutes and 72 hours.

6. A process as recited in claim 1 wherein said zinc-coated steel material is heated immediately after coating, while the coating is in a substantially molten condition, by moving said zinc-coated steel material through a continuous heating furnace.

7. A process as recited in claim 1 wherein said alloying step comprises: moving said zinc-coated steel material through a continuous heating furnace immediately after said coating step to obtain a partial amount of the desired alloying; then cooling said material; and then heating said coiled material having the partially alloyed coating in a box furnace to complete the alloying.

8. A process as recited in claim 7 wherein said coiled material is in a tightly coiled condition when it is heated in said box furnace.

9. A process as recited in claim 1 and comprising: coiling said zinc-coated steel material after coating; and performing said alloying in a box furnace.

10. A process as recited in claim 9 wherein said coil is in a tightly coiled condition when said alloying is performed in said box furnace.

**References Cited by the Examiner**

UNITED STATES PATENTS

|           |       |         |           |
|-----------|-------|---------|-----------|
| 1,307,853 | 6/19  | Dimm.   |           |
| 1,468,905 | 9/23  | Herman  | 29—196.5  |
| 1,944,227 | 9/31  | Durbin  | 117—114 X |
| 1,948,505 | 2/34  | Bray.   |           |
| 1,984,335 | 12/34 | Crapo   | 29—196.5  |
| 2,294,750 | 9/42  | Harris. |           |

|           |       |            |            |
|-----------|-------|------------|------------|
| 2,719,820 | 10/55 | Allen      | 204—37 X   |
| 2,986,808 | 6/61  | Schnedler. |            |
| 2,994,126 | 8/61  | Kennedy    | 29—196.5   |
| 3,056,694 | 10/62 | Mehler     | 29—196.5 X |
| 3,078,555 | 2/63  | McFarland  | 29—196.5   |

OTHER REFERENCES

"The Making, Shaping and Treating of Steel," 7th Edition, 1957, pages 415 and 669—672.

10 DAVID L. RECK, *Primary Examiner.*  
HYLAND BIZOT, *Examiner.*